

## UNITED STATES PATENT OFFICE.

GRANT HAMMOND, OF NEW HAVEN, CONNECTICUT.

## PROCESS FOR RECLAIMING USED PAPER.

No Drawing.

Application filed March 12, 1925. Serial No. 15,146.

*To all whom it may concern:*

Be it known that I, GRANT HAMMOND, a citizen of the United States, residing in New Haven, county of New Haven, State of Connecticut, have invented certain new and useful Improvements in Processes for Reclaiming Used Paper, of which the following is a full, clear, concise, and exact description.

This invention relates to a process for 10 claiming used paper, such as newspapers and other papers which have been printed or combined with pigments in the form of printing ink or otherwise.

The principal object of the invention is to 15 provide a simple process for reclaiming such papers which may be easily and inexpensively carried out in apparatus already in existence in paper mills and which shall produce, particularly when waste newspaper 20 stocks are used, a resulting product having superior qualities to the newspaper from which it was made.

This application is a continuation in part 25 of my application, Serial No. 697,376, filed March 6, 1924.

Broadly, the invention accordingly comprises a process for reclaiming paper having inks or pigments applied thereto, especially newspaper or similar printed paper having 30 a saponifiable binder containing the pigment, which includes beating the paper, treating it with a caustic alkali during beating and mixing an alkali acid sulfite with the resulting pulp.

In carrying out the process in its preferred form, I treat used paper, such as newspapers, in a suitable beater of the type ordinarily employed in the manufacture of paper. The amount of water employed is 35 substantially the same as that used for beating fresh pulp in paper manufacture, namely, approximately 2500 gallons per ton of paper. According to my process, this water is preferably luke warm or is heated 40 to about 110° F. and I prefer to avoid higher temperatures in most instances. I have obtained satisfactory results with temperatures as low as 80° F.

The beater is started and to it is fed 45 shredded newspaper, or other paper having a pigment thereon with a saponifiable binder such as linseed oil. Preferably during the entire beating period a solution of caustic soda is run into the paper stock. The

amount of caustic soda varies from 30 to 70 55 pounds per ton of newspaper stock but I prefer to use about 50 pounds per ton of newspaper stock, representing approximately 2.5 per cent of caustic soda based on the weight of the paper taken. This is preferably dissolved in 30 gallons of water at 60 room temperature (70° F.) and thus is added in the form of an approximately 20 per cent solution.

When the stock has been thoroughly 65 pulped, it may be washed in the beater. For this purpose I replace the caustic soda solution with cold water and continue beating. Thereafter the water is replaced by fresh 70 cold water again, and such washing may be repeated as desired.

In carrying out the whole of the reclamation process as I prefer in the beater, I next add to the washed stock, containing a fresh 75 amount of wash water (below 110° F., preferably at room temperature) equal approximately to 2500 gallons, 20 to 50 pounds of sodium acid sulfite,  $\text{NaHSO}_3$ . This material may be added in powdered form or dissolved in a small amount of water. The 80 amount of sodium acid sulfite used will depend upon the alkalinity of the pulp, enough being employed preferably to neutralize the alkali in the pulp and provide a slight excess. After the addition of sodium 85 acid sulfite, further beating of the pulp is continued until the action of the sodium acid sulfite is complete. Where the pulp contains the quantity of water which I have described 90 above, the action of the sodium acid sulfite is rapid. For one ton of pulp of a mushy consistency approximately five to twenty minutes depending upon the efficiency of the stirring apparatus employed, is sufficient to produce thorough neutralization and whitening 95 of the pulp. The same quantity of a thinner pulp, that is, one containing considerably more water may be treated to produce the same results in one to two minutes. In other words, the action of the sodium acid sulfite 100 for small quantities of pulp is substantially instantaneous and the time required mentioned above represents that necessary for sodium acid sulfite to be brought into contact with the fibers. Where smaller quantities of water are used, the pulp should be allowed to stand in contact with sodium acid sulfite, in order that its action may be

completed. The result of the action is to bleach the pulp and at the same time neutralize the alkali.

It will be understood that other alkalis than caustic soda may be used, for example, I may use caustic potash. In place of sodium acid sulphite I also may employ potassium acid sulfite.

Other kinds of paper than newspaper, 10 having a pigment printed or otherwise applied thereon with a saponifiable or like binder, may also be treated by the process.

Although I have described the entire action 15 as taking place in the beater, it is obvious that the process may be carried out in more than one vessel. For instance, I may wash the material in other beaters or stirring machines or in a rotary washer attached to the beating engine for the purpose, or 20 the pulp may be washed in separate washing machines such as are well known in the art. Instead of beating the pulp upon addition of sodium acid sulfite, I may run the pulp into storage tanks and allow the sodium acid 25 sulfite to stand in contact therewith. After treatment with the sodium bisulfite the resulting pulp may be washed to free it from excess of this material as well as from sodium sulfite and other water soluble substances. 30

The pulp so obtained may then be run out on the Foudrinier machine, formed into paper, dried, and passed through the usual 35 finishing operations. The paper so resulting is superior to the newspaper from which it was made. For example, the average news print paper shows a Mullen test of 9. Such sheets when reclaimed by my process 40 shows a Mullen test of 13. The above figures have been obtained as a result of a practical mill test on ten tons of paper. The reclaimed paper resulting from this test was not only stronger as indicated above, but was as bright in color as new unprinted news

print, and had as well, a better print surface as was demonstrated when an edition of a newspaper was printed thereon. 45

What I claim and desire to protect by Letters Patent is:

1. A process for reclaiming paper having 50 a pigment applied thereto which comprises beating the paper at a temperature below 110° F. approximately, treating it with a caustic alkali during beating and mixing an alkali acid sulfite with the resulting pulp at substantially room temperature. 55

2. A process for reclaiming newspaper which comprises beating the newspaper with water at a temperature below 110° F. approximately, treating the newspaper with 60 caustic soda during the beating, thereby producing an alkaline pulp, washing the pulp so prepared and adding at room temperature approximately a slight excess of sodium acid sulfite above that necessary to 65 neutralize the alkalinity of the pulp.

3. A process for reclaiming newspaper which comprises beating the newspaper with water at a temperature below 110° F. approximately, while running into the beater 70 a 20 per cent caustic soda solution in an amount equal approximately 2.5 per cent by weight of the newspaper taken, thereby producing an alkaline pulp, washing the alkaline pulp, adding to the washed pulp a slight 75 excess of sodium acid sulfite above that necessary to neutralize the alkalinity of the pulp, while maintaining the mass at a temperature below 110° F. approximately and washing the resulting pulp to free it from 80 excess sodium acid sulfite.

4. A process for reclaiming paper having a pigment applied thereto which comprises reducing the paper to pulp and removing the pigment therefrom, and then mixing said 85 pulp with an alkali acid sulfite at substantially room temperature.

GRANT HAMMOND.